

Jan. 20, 1931.

A. D. H. L. FASSOTTE

1,789,895

ROASTING AND/OR SINTERING OF FINE ORES OR OTHER FINE MATERIALS

Filed Nov. 17, 1927



Fig. 1



Fig. 2



Fig. 3

Inventor:  
Adolphe Louis Henri Leon Fassotte

## UNITED STATES PATENT OFFICE

ADOLPHE DENIS HENRI LÉON FASSOTTE, OF LOMMEL, BELGIUM

## ROASTING AND/OR SINTERING OF FINE ORES OR OTHER FINE MATERIALS

Application filed November 17, 1927, Serial No. 233,982, and in Belgium January 26, 1927.

This invention relates to the roasting and/or sintering of fine ores or other fine materials, more particularly of zinc ores.

It is known in processes for the roasting or sintering of sulphurous, or arsenical, or other ores, capable of reacting with air, with or without the addition of fuel, to subject the said ores on a grate to the action of drawn or blown blast. For this purpose, the contents of the ore in a heat generating element (S, As, or other) is reduced to such an extent that the temperature which is necessary for a rapid and total reaction shall be reached, without the fusing point of the ore being reached, thus keeping the reaction from suppressing the passage of the air. This result is generally obtained by a preliminary roasting, or by the mixing of materials already roasted with unroasted material.

These known processes seek to render the fine ore pervious to the air by adding water and a binding material such as clay or like material, or a combustible substance such as coal.

In all these processes, only a relative and irregular permeability of the layer of material is obtained, which implies:

The necessity of working with a very thin layer, resulting in a small output of the apparatus;

The necessity of blowing or drawing in air at a high pressure thus a high consumption of motive power and, owing to the fineness of the material, a strong tendency to the formation of holes and considerable losses of ore in the form of fine dust;

The formation of too hot and too cold regions, due to the difference of permeability, which involves either the volatilization of valuable metals or the production of an imperfectly roasted or sintered substance.

It is also known in a process of making agglomerates from fine ore, to mix the fine ore with fine fuel and to add to the mixture 30 to 35% of water to form an easily kneadable pulpy mass, which is then conveyed to an extrusion press (brick making press) adapted to form pieces of any suitable size.

These pieces are then charged into a shaft

furnace where they are heated to a sintering temperature.

In this process, the use of a shaft or high furnace implies the necessity of charging therein agglomerates of comparatively large size and of very high resistance to allow the air to pass through the column of material piled in the furnace and to prevent the crushing of the agglomerates by their own weight. This large size for the agglomerates and their great compactness, as well as the larger dimensions of the interstices make it impossible to obtain a complete roasting or uniform sintering of the ore.

The present invention contemplates a process for the roasting and/or sintering of fine ore or other fine material consisting essentially in subjecting the ore to a preparation adapted to reduce the ore to small sized grains which are afterwards subjected in a uniformly and highly pervious thin layer to a roasting and/or sintering operation on the grate of a suitable apparatus traversed by drawn or blown blast.

The ore or other fine material, brought by a preliminary operation to a suitable content in a heat generating element (sulphur, arsenic, carbon, etc.) may be subjected to a preparation and/or compression intended to impart to it a sufficient plasticity in order that by a subsequent kneading and thread-forming operation, the ore may be reduced to sufficiently resistant grains nonadherent or little adherent to each other, which grains are afterwards preferably dried and sifted, and subjected in a uniformly and highly pervious thin layer to a roasting and/or sintering operation in the manner hereinbefore stated.

By "thin layer" it is meant a layer the height of which is smaller than any of its two other dimensions.

As sintering blast apparatus provided with a grate traversed by blown or drawn blast, use may be advantageously made of the continuous apparatus called "Dwight Lloyd straight" or of the circular Von Schlippenbach apparatus, both of these apparatuses being commonly known in the art.

It is obvious that high furnaces, such as shaft furnaces cannot be used according to

55

60

65

70

75

80

85

90

95

100

the present invention, because of the small sized grains.

The fine material to be treated is preferably moistened with water before being compressed and may also be mixed with a binding material capable by drying or crystallization, and of producing the hardening of the material without destroying its perviousness during the roasting operation. The binding material should therefore, when the grains are subjected to the roasting operation, either burn (which is the case with organic binders), or become decomposed at a low temperature. As a binding material of the latter kind, sulphate of iron may be advantageously used. The sulphate of iron may be replaced by an addition of sulphuric acid to the ore, which acid produces soluble sulphates with the ore.

It is of course understood that the utilization of sulphate of iron, sulphuric acid or any other binding material when roasting fine ore is known "per se" and that I do not claim these binding materials as forming my invention. It is in fact possible to do away with the addition of a binding material by effecting a preliminary sulphatizing roasting or by leaving the moist material exposed for a certain time to the action of the atmospheric agents.

By way of example, a mode of carrying the invention into effect when applied to a dead roasting of blonde, is given hereinafter:

The blonde subjected to a preliminary roasting until the contents of sulphur are brought to the desired amount (5 to 7%) or brought by mixing to a contents of sulphur or other combustible material corresponding to the same calorific power as 3 to 6% of sulphur in sulphide form, and mixed with 1 to 5% of sulphate of iron and 5 to 25% of water, is fed into a kneading-threadforming apparatus.

The accompanying drawings illustrate diagrammatically and by way of example, an apparatus which may be advantageously used for carrying the process into practice.

Fig. 1 shows the whole of the apparatus in a longitudinal vertical section;

Fig. 2 is a plan view corresponding to Fig. 1; and

Fig. 3 is an elevation on a large scale, of the kneading-threadforming apparatus.

Having more particular reference to the drawings, wherein like characters of reference will designate corresponding parts throughout, the apparatus may be stated to comprise a tubular mixing body 1 terminated by a conical flaring portion 1' followed by a cylindrical body of larger diameter 2.

Extending longitudinally through the bodies 1 and 2, is a rotatable shaft S carrying at one end a plurality of radially disposed blades 3 adapted to propel the material while mixing and kneading the same. Arranged

upon the intermediate portion of the shaft, are two screws 4 and 5 causing the material to advance while being compressed. Upon the other end of the shaft S are arranged two or more radial blades 6 preferably curved at their free edges in an opposite direction to the movement of rotation of the shaft.

The lower portion of the cylindrical body 2 carries a perforated sieve 2' having perforations measuring from 3 to 5 mm. in diameter, preferably 3½ or 4 mm. for the ordinary blends.

The material which arrives kneaded and compressed in the cylindrical portion, is forced by the blades through the sieve and falls in the form of short and rather breakable thin cylinders into the conveyor 7, these cylinders dividing themselves into small pieces of various lengths. The most favourable size for the grains is comprised between 3 and 4 mm. diameter. The length of the grains may vary within larger limits, from 2 to 15 mm. for instance.

The conveyor moves through suitable driving mechanism with a continuous motion, carrying, in the form of a thin and regular layer, the material which is continuously produced by the two kneading-threadforming devices 8 and penetrates inside a tunnel or other drying device 9 kept by a furnace 10 or other source of heat at a suitable temperature. The grains leave dryer in a hardened and more or less completely dried state and fall into a sifting apparatus consisting of two superposed sieves, the upper one 11 having meshes of approximately 10 mm., and the lower one 12 having meshes of approximately 2 mm. A roller 13 disintegrates any eventual conglomerates of grains which may have been formed during the drying operation.

The granulated material, deprived of fine dust, falls from the sieve 12 into a storing hopper 14 which distributes it uniformly upon the grate 15 of the blast apparatus which is displaced underneath it. It should be noted that if the grains, as said above, are subjected to a drying operation, this drying is only necessary up to the desired point for obtaining grains capable of being sifted for eliminating the dust and of being charged onto the grate without the formation of a new amount of dust. If in the threadforming operation grains are obtained which are well compressed, having a little or nonadhering surface, deprived of dust and capable of being subjected to a cautious charging operation, without disintegration, it is possible to charge the material direct onto the grate of the blast apparatus without a preliminary drying operation. If not, the drying operation will be effected more or less completely according to circumstances; it may even be only superficial and of short duration. It is also possible to effect a mixed charging of

superposed layers of non-dried, semi-dried and dried grains.

5 The amount of sulphur or other heat-generating element to be left or introduced into the ore depends on the degree of dryness of the latter; it will be minimum in the case of a complete dryness; for the blonde it will be about 5% of sulphur in sulphide form.

10 The present process enables to obtain numerous and important advantages, due essentially to the high and uniform perviousness of the layer of small-sized grains which are used.

The main advantages are:

15 1. The desulphurization is effected very thoroughly and the amount of sulphur which remains in the mass is negligible. It may fall for normal blenders as low as 0.10%.

20 2. The pressure or depression necessary for the apparatus with forced or drawn blast is reduced, resulting in a saving of motive power and reduction to a large extent, of the air admission which occurs with apparatuses having movable joints. By way of example, 25 for a layer of 0.25 m. thickness of grains of 3.5 mm. diameter the depression may vary between 7 and 3 cm. of water.

30 3. The granulated material may be dry and does not require any addition. It has no tendency to the formation of holes through the action of the blast. For the same reasons, the carrying away of material during the passage of blast is practically nil.

35 4. The thickness of the layer placed on the blast apparatus may be considerably higher than with nongranulated material whence the costs of ignition are decreased in proportion; a thickness of 0.50 m. should however be considered as being near to the limit which 40 cannot be exceeded in practice owing to the difficulties arising from an increased pressure or vacuum and to the danger of having the grains crushed by their own weight; moreover the reaction progresses much more 45 rapidly than with non granulated material, whence an increase of the output of the apparatus to very large proportions.

50 5. The gas which is obtained is for these reasons, comparatively rich in sulphur dioxide,  $\text{SO}_2$  (in the case of blonde roasting 3 to 5% of sulphur dioxide,  $\text{SO}_2$  can be obtained with a blast apparatus which is well constructed from the point of view of tight-joint fit); the gas is on the other hand practically free from water vapour and this is indispensable for certain processes of manufacture of sulphuric acid.

55 6. An even temperature at all points is obtained without having too hot zones where semi-fusings are produced with abundant volatilization of useful metals (zinc, lead, etc.) and cold zones in which the roasting or sintering is incomplete.

60 7. Lastly, it is possible to adjust the amount of heat-producing substances (sul-

phur in the case of blenders) and to conduct the blast delivery in such a manner as to obtain a completely roasted product without fusing, scorification or even fritting of the material, in such a manner that after roasting, the grains are obtained almost intact in shape, porous and easily separable from each other without a troublesome production of dust, the material thus obtained being in a state which is highly favourable for the subsequent operations and more particularly for obtaining the reduction of the zinc ores in the zinc oven.

I claim:

1. In a process for the roasting of fine ore material in the form of a comparatively thin layer, the preliminary steps of subjecting the said ore material to a mixing-threadforming operation, whereby threads having all the same small diameter are expressed in a practically vertical direction against a conveyor band which is uniformly moved without shaking, and are bent by the movement of the conveyor band so that they break into short pieces having the same small diameter and approximately same length, allowing the said short pieces to dry before disturbing them for the blast roasting operation, as set forth.

2. In a process for the roasting of fine zinc ore material in the form of a comparatively thin layer, the preliminary steps of subjecting the said zinc ore material to a preliminary mixing-threadforming operation, whereby threads having all the same small diameter are expressed in a practically vertical direction against a conveyor band which is uniformly moved without shaking, and are bent by the movement of the conveyor band so that they break into short pieces having the same small diameter and approximately same length, allowing the broken pieces to dry before disturbing them for the blast roasting operation, as set forth.

ADOLPHE DENIS HENRI LÉON FASSOTTE.

110

115

120

125

130